

## UNITED STATES PATENT OFFICE

2,458,442

FOG INHIBITOR FOR PHOTOGRAPHIC  
EMULSIONS

Robert Eliot Stauffer and William F. Smith,  
Rochester, N. Y., assignors to Eastman Kodak  
Company, Rochester, N. Y., a corporation of  
New Jersey

No Drawing. Application October 17, 1947,  
Serial No. 780,568

12 Claims. (Cl. 95—7)

1

This invention relates to fog-inhibiting agents and stabilizers for photographic emulsions and to photographic emulsions containing them.

It is known that photographic emulsions, particularly ultra-sensitive emulsions or those containing optical sensitizers exhibit a tendency to form a deposit of silver in the emulsion. This deposit extends more or less uniformly over the entire emulsion and is known as fog. Photographic fog is of two types: local and general. Local fog is formed by exposure of the film or plate at undesired points as by a light leak in the camera. General fog is formed in a number of ways. It may be caused by the conditions under which the film or plate is stored such as conditions of high temperature or humidity or unusually long time of storage. The nature of the emulsion may also produce general fog as well as the conditions of development of the emulsion as by development for protracted periods of time or at temperatures above normal. We are primarily concerned with the fog and sensitivity changes in films or plates which have been stored under adverse conditions of temperature and humidity.

General fog and loss of sensitivity of the emulsion are especially likely to occur when the sensitive material is stored under conditions other than ideal, that is, under conditions of high temperature and humidity as in tropical regions.

It is an object of the invention to provide novel anti-fogging or fog-inhibiting compounds for emulsions. A further object is to provide anti-fogging agents which stabilize the initial sensitivity of the emulsion. A still further object is to provide anti-fogging agents which improve the keeping of the emulsion in tropical regions. Other objects will appear from the following description of our invention.

These objects are accomplished by incorporating in a silver halide emulsion an acid or a salt having the general formula:



in which R is hydrogen, ammonium or an alkali metal. X is a halogen atom, and Re is the element rhenium.

Compounds suitable for use according to our invention are those of the above general formula, in which R is hydrogen, ammonium or an alkali

2

metal such as sodium or potassium and X is a halogen atom such as chlorine, bromine or iodine. Suitable compounds are potassium chlororhenate,  $K_2ReCl_6$ ; potassium bromo rhenate,  $K_2ReBr_6$  and potassium iodorhenate,  $K_2ReI_6$ .

The object of our invention is to maintain the sensitivity and fog of silver halide emulsions at or close to initial optimum values under keeping conditions of high temperature and humidity.

10 The fog inhibitors which we propose to use are added to the emulsion during the process of manufacture to avoid loss of sensitivity and to inhibit the growth of fog with passage of time under non-ideal conditions of storage.

15 A solution of  $R_2ReX_6$  compound when added in suitable concentration before coating to unsensitized or optically sensitized photographic emulsions does not appreciably affect the sensitometric values for sensitivity and fog when measurements are made soon after coating. When sensitometric measurements are made at appreciable intervals of time under tropical or dry conditions of storage at elevated temperatures, however, this compound does stabilize photographic speed and maintain fog at a low level.

20 The preparation of silver halide emulsions involves three separate operations (1) the emulsification and digestion or ripening of the silver halide, (2) the freeing of the emulsion from excess soluble salts usually by washing, (3) the second digestion or after-ripening to obtain increased sensitivity. (Mees, The Theory of the Photographic Process, 1942.) We prefer to add the fog-inhibiting agents after the final digestion

25 or after-ripening although they may be added before digestion. The most useful concentration range of fog inhibitor is from .26 to 3.9 gm. of fog inhibitor per kilogram of silver nitrate used in making the particular silver halide emulsion and 30 converted to silver halide. The quantity used will of course vary for example depending on the silver halide or mixture of halides used.

35 The anti-fogging and stabilizing action was determined by incubation of the emulsions under simulated tropical conditions and also by incubation at low relative humidity at 120° F. for various lengths of time from 12 days to one month. The results of these tests are tabulated here and are compared with the initial speed, gamma and fog of the emulsions with and without the anti-

foggant and stabilizing compound. The tests from which the following tabulation was made used a high-speed silver bromoiodide emulsion exposed on an Eastman type IIB sensitometer and developed for five minutes in a developer of the following composition:

|                                   | Grams |
|-----------------------------------|-------|
| Monomethyl paraminophenol sulfate | 2.5   |
| Sodium sulfite (desiccated)       | 30.   |
| Hydroquinone                      | 2.5   |
| Sodium metaborate                 | 10.   |
| Potassium bromide                 | 0.5   |
| Water to one liter.               |       |

The results for  $K_2ReCl_6$  are as follows:

| Gms. of compound /Kg. $AgNO_3$ (converted to $AgX$ ) used in emulsion | Original   |       |     | 12 Days at 120° F. |       |     | 1 Mo. Tropical |       |     |
|-----------------------------------------------------------------------|------------|-------|-----|--------------------|-------|-----|----------------|-------|-----|
|                                                                       | 10/l speed | Gamma | Fog | 10/l speed         | Gamma | Fog | 10/l speed     | Gamma | Fog |
| None.....                                                             | 455        | 1.41  | .20 | 455                | 1.44  | .25 | 203            | 1.56  | .20 |
| .26.....                                                              | 465        | 1.37  | .20 | 540                | 1.37  | .26 | 200            | 1.51  | .21 |
| .52.....                                                              | 425        | 1.40  | .14 | 615                | 1.30  | .20 | 255            | 1.43  | .13 |
| 1.30.....                                                             | 345        | 1.46  | .14 |                    |       |     | 162            | 1.63  | .14 |

One of the advantages of our invention is the fact that compounds such as  $K_2ReCl_6$  are readily prepared with high purity.  $K_2ReCl_6$  is prepared and may be used as follows:

The compound was prepared by intimately mixing powdered potassium chloride and rhenium metal, and fusing carefully at dull red heat in a silica tube and silica combustion boat in a current of dry chlorine gas. The temperature was not allowed to go too high in order to prevent sublimation of rhenic chloride from the tube. After cooling in a chlorine atmosphere, the greenish yellow sintered mass was dissolved in water, filtered to remove unreacted metal and carefully crystallized by concentration at room temperature over sulfuric acid in a vacuum desiccator. The crystals of  $K_2ReCl_6$  were pale green showing a high index of refraction and high dispersion. They appear isomorphic with  $K_2PtCl_6$  (potassium hexachloroplatinate). The rhenium complex was dissolved in water at a convenient concentration and was added to a melted gelatinous silver bromo-iodide photographic emulsion in quantities ranging up to about 3.9 grams per kg. of  $AgNO_3$  (converted to  $AgX$ ) in the emulsion. The emulsion was coated on a suitable support, glass, film, or other, and was dried in the normal way. The other  $R_2ReX_6$  compounds may be prepared and used in a similar manner.

Another and perhaps chief advantage is the greater extent of stabilizing action over a wide range of climatic conditions.

The fog inhibiting agents which we have described may be used in various kinds of photographic emulsions. In addition to being useful in ordinary non-sensitized emulsions they may also be used in orthochromatic, panchromatic and X-ray emulsions. If used with sensitizing dyes, they may be added to the emulsion before or after the dyes are added. Various silver salts may be used as the sensitive salt such as silver bromide, silver iodide, silver chloride and mixtures of these. The dispersing agents may be gelatin or other colloid such as collodion, albumen, cellulose organic derivatives or synthetic resins.

We also contemplate as a part of our invention those cases where it is desirable to coat the antifoggant in a colloid layer such as gelatin on either or both sides of or also in a silver halide emulsion layer, so that the antifoggant is con-

tiguous to the silver halide emulsion. In these cases we use the same or a slightly greater ratio of rare metal salt to silver halide as when the salt is in the emulsion layer.

It will be understood that we contemplate as included within our invention all modifications and equivalents falling within the scope of the appended claims.

What we claim is:

1. A silver halide emulsion layer containing a compound having the structure



where  $X$  is a halogen atom and  $R$  is of the group consisting of hydrogen, ammonium and alkali metals.

15

2. A silver halide emulsion layer containing a compound having the structure



where  $X$  is a halogen atom and  $R$  is of the group consisting of hydrogen, ammonium and alkali metals, said compound being present in said emulsion layer in a concentration of from 0.26 to 3.9 grams per kilogram of silver nitrate used in making said emulsion and converted to silver halide.

35 3. A silver halide emulsion layer containing a compound having the structure



40 where  $R$  is of the group consisting of hydrogen, ammonium and alkali metals.

4. A silver halide emulsion layer containing a compound having the structure



45 where  $R$  is of the group consisting of hydrogen, ammonium and alkali metals.

5. A silver halide emulsion layer containing a compound having the structure



50 where  $R$  is of the group consisting of hydrogen, ammonium and alkali metals.

6. A silver halide emulsion layer containing a compound having the structure



where  $R$  is an alkali metal.

7. A silver halide emulsion layer containing a compound having the structure



65 where  $R$  is an alkali metal.

8. A silver halide emulsion layer containing a compound having the structure



70 where  $R$  is an alkali metal.

9. A silver halide emulsion containing potassium chlororhenate.

10. A silver halide emulsion containing potassium bromorhenate.

11. A silver halide emulsion containing potassium iodorhenate.

75

12. A light sensitive photographic element comprising a silver halide emulsion layer and a colloid layer contiguous to said emulsion layer, at least one of said layers containing a compound having the structure

$R_2ReX_6$

where **X** is a halogen atom and **R** is of the group consisting of hydrogen, ammonium and alkali metals.

ROBERT ELIOT STAUFFER.  
WILLIAM F. SMITH.

No references cited.